

1

3,310,170

## SYLVINITE FLOTATION WITH AMINE COMPOSITION

Charles W. Abernethy and Milton H. Klein, Carlsbad, N. Mex., assignors to American Metal Climax, Inc., New York, N.Y., a corporation of New York  
No Drawing. Filed May 18, 1964, Ser. No. 368,405  
9 Claims. (Cl. 209—166)

This invention relates to the beneficiation of sylvite ores to produce concentrated sylvite values. More particularly, the present invention relates to the concentration of sylvite values from sylvite ores by froth flotation employing improved cationic sylvite collecting reagents.

It has, of course, been known heretofore to employ froth flotation reagents to effect the concentration of desired mineral values. More specifically, it has been known to employ aliphatic fatty acid amine salts, and, illustratively, primary aliphatic amine salts wherein the hydrocarbon moieties contain at least eight carbon atoms, as sylvite collectors.

It has also been suggested hitherto to enhance the effectiveness of fatty acid amine collector salts by increasing or decreasing the degree of unsaturation in concert with the temperature of the brine solute in which the pulp is suspended. This procedure, however, involves obvious disadvantages inherent in correlating hydrogenation of the hydrocarbon portions of the amines involved with the consistently varying temperatures which normally occur in the environments wherein these froth flotation procedures are performed. To control the temperature of this environment would, on the other hand, be unduly costly.

It has now been discovered, however, that a unique and selective mixture of primary saturated (mostly) amine salts may be had which will provide a significantly improved and efficient sylvite collecting reagent at ambient temperatures. Accordingly, the present invention is based on the discovery that a pulp formed from comminuted sylvite ore suspended in a brine saturated with the constituents of said ore is most effectively conditioned for froth flotation at ambient temperatures by introduction therein of a cationic mineral collector composition composed of 60 percent to 80 percent, and desirably 65 percent to 75 percent, of the acid addition salts of hydrogenated tallow amine and 40 percent to 20 percent, and preferably 35 percent to 25 percent, respectively, of cocoa amine salt and most desirably one formed from 75 percent of hydrogenated tallow amine salt and 25 percent of cocoa amine salt, having an iodine value preferably below 12.

The foregoing preferred cationic amine composition (i.e. a mixture of about 75 percent hydrogenated tallow amine salt and 25 percent cocoa amine salt) contains the primary normal or unbranched saturated and olefinitely slightly unsaturated aliphatic fatty acid amines having from 8 to 18 carbon atoms in the approximate percentages by weight indicated in Table I.

TABLE I

| Name     | No. of Carbons | No. of Double Bonds | Percent |
|----------|----------------|---------------------|---------|
| Caprylyl | 8              | None                | 1.5     |
| Capryl   | 10             | do                  | 1.8     |
| Lauryl   | 12             | do                  | 13.5    |
| Myristyl | 14             | do                  | 6.0     |
| Palmityl | 16             | do                  | 25.1    |
| Stearyl  | 18             | do                  | 46.6    |
| Oleyl    | 18             | One                 | 5.2     |
| Linoleyl | 18             | Two                 | 0.3     |

The foregoing amines are, as indicated, employed in the form of their corresponding acid addition salts prepared in the usual manner by reaction of the amines with suitable acids such as sulfuric acid, phosphoric acid,

2

the hydrohalic acids, e.g. hydrobromic acid and hydrochloric acid, or acetic acid. In this manner the amine collecting reagents of the invention are rendered water-soluble.

5 The effectiveness of the flotation step is influenced significantly by the chain lengths of the hydrocarbon, i.e. alkyl and alkenyl, radicals present in the hydrogenated tallow amine and cocoa amine salts, and the relative proportions of the various chain lengths within the range recited, i.e. 8 to 18 carbon atoms, when inter-related with the primary saturation of the components. Although not narrowly critical, the preferred concentration of cationic collector per ton of the comminuted ore feed is .07 pound to .16 pound. The preferred particle sizes of comminuted ore to which the instant amine reagents are applied are of minus 8 mesh.

10 The nonmetallic mineral ores subject to the practice of the present invention are particularly those potash ores containing mixtures of oceanic salts and clays of which sylvite (potassium chloride) is a normal constituent. A major and illustrative source of sylvite (KCl) in North America is the mineral deposits of the Permian Basin, and particularly those occurring in the vicinity of Carlsbad, N. Mex. Other known sources of suitable ore deposits are those present in California, Utah and Saskatchewan, Canada.

15 The sylvite ore is characteristically subjected, after being mined, to a preliminary crushing, employing conventional grinding apparatus, and is sequentially comminuted by passage thereof through a hammermill, pebble mill, or by impact pulverization to liberate the sylvite constituents of the ore. Comminution of the ore is indeed preferably carried out by impact pulverization with substantially dry ore. The resulting mill feed is then, 20 in one illustrative procedure, admixed with a brine solution saturated with the constituents of the sylvite ore and suspended in the brine to provide a pulp which is then subjected to various forms of violent agitation in a scrubbing operation wherein substantial quantities of the clay slimes present in the ore are released from the salt crystals therein and suspended in the brine which is then removed. Thereafter the sylvite pulp is passed to sizing and classifying apparatus employing such conventional equipment as cyclones, rake and bowl classifiers, wet or 25 dry stationary or vibrating screens, settling cones, hydroseparators, and the like.

25 In the classifying operation at least two fractions of pulp are prepared; one containing, for example, undersize particles of 65 mesh or finer and a second fraction of plus 65 mesh. The former fraction containing the undersize or fine particles of sylvite also contains considerable quantities of residual slimes which are partially and conveniently removed suspended in brine as overflow from hydroseparators. The brine of this overflow, which is 30 saturated with sylvite ore constituents, is normally separated from the foregoing slimes and recycled for use with another portion of mill feed. The remaining fraction or fractions containing coarser or oversize particles of comminuted ore are normally combined thereafter with the partially deslimed first fraction of undersize ore particles and the resulting pulp is then conditioned for the froth flotation steps to follow.

35 Conditioning is effected by introduction into the pulp of the amine reagent composition of the present invention as described hereinabove, preferably in the amount and concentration indicated, followed by agitation of the resulting mixture. This agitation is accomplished either mechanically or by means of a current of air or other unreactive gas. The cationic conditioning or collecting compositions of the invention may be introduced into contact with the pulp either directly or, if desired, with water-immiscible oils, such as pine oil, fuel oil, or kero-

sene, or with a frothing reagent of commercial grade, such as methyl isobutyl carbinol, which cooperate with the cationic amine salt flotation reagents of the invention. Flotation oils, where included, are usually not introduced in excess of .08 pound thereof per ton of mill feed; a desirable range, in such instances, being from 0.03 to .06 pound per ton of sylvite mill feed.

Due to the uneconomic and impractical mechanical methods presently available for effecting complete removal of clay slimes from the pulp, there is introduced, usually in the conditioning step, prior to conditioning with the collector, an auxiliary reagent to inhibit the adverse effect of the residual slimes upon the collection, particularly of the coarser values, in the froth flotation step or steps.

Illustrative of such inhibiting reagents are starch, dextrin, the polyglycols and their ethers disclosed in Patent 2,724,499 of Smith et al., and the water-soluble acrylonitrile polymers of Patent 2,919,026 of Smith et al.; that is, by way of further illustration, a water-soluble acrylonitrile polymer in which at least one nitrile group has been modified by alcoholysis to produce the corresponding ester and/or alkaline hydrolysis to produce the corresponding salt.

Where the auxiliary reagent is a polyglycol or polyglycol ester having a molecular weight of at least 300 the quantity of reagent employed is at least 0.08 pound per ton of the ore initially submitted to the process as mill feed. In like manner, where a water-soluble acrylonitrile polymer is utilized as an auxiliary reagent, the concentration thereof is at least 0.02 pound per ton of sylvite mill feed.

It will be evident, too, that other standard conditioning and cooperating reagents known heretofore may be additionally introduced, optionally, in known concentrations, in the sylvite pulp to be subjected to froth flotation in accordance with the practice herein described.

The actual froth flotation, which is most desirably accomplished in deep air cells of standard manufacture, can also be effected in any of a variety of other means, such as Denver Equipment Company cells, Mineral Separation cells, Forrester Air-Lift cells, and Turbo-cells, as well as in laboratory models, such as the Fagergren flotation machine.

In one illustrative method, the pulp is subjected to a plurality or sequence of flotation operations, such, for example, as an initial rougher flotation, a cleaner flotation, and a recleaner flotation, which are standard procedures well-known in the art. It will be evident that the froth flotation techniques, wherein the cationic sylvite collectors of the present invention are employed, may be widely varied. Thus, for example, the fine fraction containing ore particles of 65 mesh or finer, and the other fraction or fractions containing particles of plus 65 mesh resulting from the sizing and classifying means employed, may

be separately treated with the conditioning reagents of the invention; or, indeed, a fraction containing the coarser particles may be admixed initially, separately and solely, with the cationic collectors here involved, subjected to a rougher flotation separately, and the rougher concentrate recovered therefrom then subjected to a cleaner flotation in admixture with the fine pulp fraction, the amine collector introduced in the foregoing conditioning step having been provided in an amount sufficient to serve effectively for collection of the sylvite values in both the rougher and cleaner flotations and, for that matter, if desired, in any recleaner flotation step to follow. Accordingly, an illustrative procedure wherein the cationic sylvite collecting compositions of the present invention can be employed is described in copending application Ser. No. 320,388 now Patent Number 3,282,418 filed by the applicants herein on October 31, 1963.

The following examples are further illustrative of the invention.

#### Example 1

Twelve samples of a sylvite ore mined in the Carlsbad, New Mexico region, each containing about 23% K<sub>2</sub>O equivalent of potassium chloride (see table), are comminuted after initial crushing by impact pulverization to provide a mill feed. Each of the mill feeds is subjected, individually and sequentially, to scrubbing for the purpose of effecting preliminary desliming after introduction of a brine, having a specific gravity of about 1.240, and previously saturated with the constituents of sylvite ore, to form a pulp. The pulp submitted to the aforesaid scrubbing operation contains about 60 percent by weight of suspended solids. The pulp resulting from the foregoing preliminary desliming operation, in each instance, is thereafter classified into two fractions of about 15 percent 65 mesh or finer and 85 percent plus 65 mesh by standard procedures. The finer pulp of each sample processed, containing particles of 65 mesh or finer, is further deslimed in standard hydroseparators and then admixed with the coarser fraction of plus 65 mesh, and each of the resulting compositions is then subjected to conditioning in the manner and with the reagents, in the concentrations and amounts indicated, in Table II. The efficiency of the flotation recovery procedure employing the cationic amine salt collector reagents indicated is also represented in Table II. The cationic amines employed in the form of their acid addition salts, which are chemically unreactive with the constituents of the sylvite ore, added to the respective samples as indicated, i.e. (a) to (l), are represented by the symbols in Table II having the following significance:

- A. distilled tallow amine hydrochloride
- B. distilled hydrogenated tallow amine hydrochloride
- C. cocoa amine hydrochloride, distilled and saturated

TABLE II

| Sample No. | Amine Used              | Rate, Lbs./Ton of Mill Feed | Percent K <sub>2</sub> O |             |      | Recovery, Percent of K <sub>2</sub> O Equivalent |
|------------|-------------------------|-----------------------------|--------------------------|-------------|------|--------------------------------------------------|
|            |                         |                             | Feed                     | Concentrate | Tail |                                                  |
| (a)-----   | A-----                  | .07                         | 23.45                    | 58.45       | 6.44 | 81.52                                            |
| (b)-----   | { 60% B<br>40% C }----- | .07                         | 23.19                    | 59.28       | 3.59 | 89.83                                            |
| (c)-----   | { 70% B<br>30% C }----- | .07                         | 23.30                    | 59.46       | 2.99 | 91.78                                            |
| (d)-----   | B-----                  | .07                         | 23.05                    | 54.04       | 6.35 | 82.09                                            |
| (e)-----   | A-----                  | .13                         | 23.27                    | 50.08       | 3.81 | 89.39                                            |
| (f)-----   | { 40% B<br>60% C }----- | .13                         | 23.09                    | 50.01       | 2.27 | 93.78                                            |
| (g)-----   | { 60% B<br>40% C }----- | .13                         | 23.10                    | 59.15       | 1.25 | 96.63                                            |
| (h)-----   | { 70% B<br>30% C }----- | .13                         | 23.04                    | 59.45       | 1.09 | 97.11                                            |
| (i)-----   | A-----                  | .16                         | 23.06                    | 58.47       | 2.11 | 94.25                                            |
| (j)-----   | { 35% B<br>65% C }----- | .16                         | 23.29                    | 58.34       | 2.55 | 93.12                                            |
| (k)-----   | { 60% B<br>40% C }----- | .16                         | 23.02                    | 58.61       | 1.18 | 96.81                                            |
| (l)-----   | A-----                  | .22                         | 22.98                    | 57.98       | 1.41 | 96.21                                            |

The procedure of this example is carried out at ambient temperatures, which in each of the foregoing instances is about 70° F.

Percentages in the foregoing Table II as well as throughout this specification refer to percentages by weight unless otherwise explicitly indicated.

The marked enhancement in efficiency of the flotation recovery in those instances where a mixture of hydrogenated distilled tallow amine hydrochloride and distilled cocoa amine hydrochloride within the proportions of the invention are employed, i.e. with samples (b), (c), (g), (h) and (k), over those instances where a hitherto known flotation reagent, distilled tallow amine hydrochloride, i.e. ore samples (a), (e), (i) and (l); hydrogenated distilled tallow amine hydrochloride, i.e. sample (d); or even mixtures of hydrogenated distilled tallow amine hydrochloride and distilled cocoa amine hydrochloride in proportions outside of those of the invention, i.e. samples (f) and (j), are utilized, is readily evidenced in the foregoing Table II. The particularly effective performance of the preferred sylvite collector composition composed of 70 percent hydrogenated tallow amine salt and 30 percent saturated cocoa amine salt is also manifested in the foregoing Table II. It will be seen, too, that employment of compositions envisioned by the present invention, i.e. the flotation collection reagents utilized in treatment of the pulp samples (h) and (k), at a rate of 0.13 to 0.16 pound per ton of mill feed, results in a superior flotation recovery to that of 0.22 pound of distilled tallow amine hydrochloride per ton of mill feed as manifested in the treatment of pulp sample (1).

Before hydrogenation the distilled tallow amine hydrochloride of the foregoing Example 1 and Table II, employed for purposes of comparison with the compositions coming within the purview of the invention, has the approximate composition recited in Table III; the amines reported therein being employed in Example 1, as indi-

5 10 15 20 25 30 35

5. In this instance, unsaturated moieties of the various amine components normally have up to 2 percent of unsaturated aliphatic amine components as compared to 42.5 percent of such unsaturated components in the aforesaid unhydrogenated, distilled tallow amine and its corresponding salts.

#### Example 2

The procedure of Example 1 was repeated but in this instance was carried out on a full-scale plant operation employing seven ore portions averaging over 50,000 tons each. The procedure employed varied, too, in the temperature of the brine in which the ore particles of the samples were in each instance suspended. Thus, the processing of samples (m), (n), (o), and (p), as recited in Table IV appearing hereinafter, was carried out within a brine temperature range of 72° F. to 89° F. inclusive, while the processing of ore samples (q), (r), and (s), as recited in Table V appearing hereinafter, was carried out within a brine temperature range of 59° F. to 68° F. inclusive. The symbols employed in Tables IV and V to indicate the particular amine conditioning reagent used with the respective ore samples are identical with those recited in Example 1, i.e. A represents distilled tallow amine hydrochloride; B indicates hydrogenated distilled tallow amine hydrochloride; and C symbolizes saturated and distilled cocoa amine hydrochloride. These tables further indicate the concentrations of the amine reagents employed with each of the foregoing samples and the efficiency of the flotation recovery secured in each instance.

TABLE IV

| Sample No. | Amine Used                 | Rate, Lbs./Ton of Mill Feed | Percent K <sub>2</sub> O |             |      | Recovery, Percent of K <sub>2</sub> O Equivalent |
|------------|----------------------------|-----------------------------|--------------------------|-------------|------|--------------------------------------------------|
|            |                            |                             | Feed                     | Concentrate | Tail |                                                  |
| (m)-----   | A-----                     | .152                        | 22.66                    | 55.41       | 1.92 | 94.81                                            |
| (n)-----   | {75% B-----<br>25% C-----} | .118                        | 24.23                    | 55.29       | 1.86 | 95.54                                            |
| (o)-----   | {75% B-----<br>25% C-----} | .117                        | 23.33                    | 56.48       | 1.78 | 95.38                                            |
| (p)-----   | A-----                     | .155                        | 23.89                    | 55.92       | 1.71 | 95.77                                            |

TABLE V

| Sample No. | Amine Used                 | Rate, Lbs./Ton of Mill Feed | Percent K <sub>2</sub> O |             |      | Recovery, Percent of K <sub>2</sub> O Equivalent |
|------------|----------------------------|-----------------------------|--------------------------|-------------|------|--------------------------------------------------|
|            |                            |                             | Feed                     | Concentrate | Tail |                                                  |
| (q)-----   | A-----                     | .150                        | 23.05                    | 55.90       | 1.48 | 96.12                                            |
| (r)-----   | {68% B-----<br>32% C-----} | .126                        | 22.71                    | 56.73       | 1.57 | 95.74                                            |
| (s)-----   | A-----                     | .146                        | 22.87                    | 56.58       | 2.01 | 94.57                                            |

cated, in admixture in the form of their hydrochloride salts.

TABLE III

| Primary Amine    | No. of Carbons | No. of Double Bonds | Percent |
|------------------|----------------|---------------------|---------|
| Myristyl-----    | 14             | None                | 3.0     |
| Pentadecyl-----  | 15             | None                | 0.5     |
| Palmityl-----    | 16             | None                | 29.5    |
| Margaryl-----    | 17             | None                | 1.0     |
| Stearyl-----     | 18             | None                | 23.5    |
| Myristoleyl----- | 14             | 1                   | 1.0     |
| Palmitoleyl----- | 16             | 1                   | 3.0     |
| Oleyl-----       | 18             | 1                   | 37.0    |
| Linoleyl-----    | 18             | 2                   | 1.5     |

65 It will be evident from the comparative studies of foregoing Example 2 that the significant and superior efficacy of the cationic sylvite collectors of the invention employed with Samples (n), (o), and (r) in the foregoing Tables IV and V is sustained over a comparatively broad range of brine temperatures.

Accordingly, it will be apparent that the present invention provides cationic mineral collectors of unexpected efficiency for effecting the recovery of sylvite from sylvanite ores.

The criticalness of the increased efficiency in concentration of sylvite values effected by the sylvite collectors of the invention as manifested in the foregoing examples 70 is particularly evident when viewed in terms of the vast

quantities of sylvanite ores mined and the criticalness of cost in the processes involved.

Various modifications of the invention may occur, and to the extent that such modifications and variations incorporate the spirit of this invention, they are intended to be included within the scope of the appended claims.

What is claimed is:

1. A process for effecting the froth flotation of sylvanite ore that comprises comminuting said ore, forming a pulp containing said comminuted ore suspended in a brine saturated with the constituents of the ore and agitating said pulp containing said sylvanite ore in comminuted condition in the presence of a cationic sylvite collector composed of a mixture of 65 percent to 75 percent by weight of an acid addition salt of hydrogenated distilled tallow amine and 35 percent to 25 percent, respectively, of an acid addition salt of distilled cocoa amine, said mixture having an iodine value of less than 12.

2. A process for separating sylvite values from pulp formed of particles of comminuted sylvanite ore suspended in a brine saturated with the constituents of said ore that comprises subjecting said pulp to a froth flotation process employing as the cationic sylvite collector, a mixture of 70 percent by weight of an acid addition salt of hydrogenated distilled tallow amine and 30 percent of an acid addition salt of distilled cocoa amine, said mixture having an iodine value of less than 12; and said mixture being employed in an amount of 0.07 to 0.16 pound per ton of said ore.

3. A process for separating sylvite values from a pulp composed of a mill feed of comminuted sylvanite ore suspended in a brine saturated with the constituents of said ore that comprises subjecting said pulp to a froth flotation process employing as the cationic sylvite collector, a mixture of acid addition salts of the primary unbranched, saturated and olefinically unsaturated aliphatic amines, caprylyl amine, capryl amine, lauryl amine, myristyl amine, palmityl amine, stearyl amine, oleyl amine, and linoleyl amine in percentages by weight, respectively, of about 1.5 percent, 1.8 percent, 13.5 percent, 6.0 percent, 25.1 percent, 46.6 percent, 5.2 percent and 0.3 percent; said mixture having an iodine value of less than 12; and said mixture being employed in an amount by weight .07 to .16 pound per ton of said mill feed; said process being conducted at ambient temperatures.

4. The process of claim 3 wherein the process is carried out at a temperature within the range of 60° F. to 90° F.

5. A froth flotation composition comprising a pulp composed of comminuted sylvanite ore suspended in a brine saturated with the constituents of said ore; and admixed therewith, a cationic sylvite collector composed of a mixture of 60 percent to 80 percent by weight of an acid addition salt of hydrogenated tallow amine and 40 percent to 20 percent, respectively, of an acid addition salt of distilled cocoa amine, said mixture having an iodine value of less than 12.

6. A forth flotation composition comprising a pulp

composed of comminuted sylvanite ore suspended in a brine saturated with the constituents of said ore; and admixed therewith, a cationic sylvite collector composed of a mixture of 65 percent to 75 percent by weight of an acid addition salt of hydrogenated distilled tallow amine and 35 percent to 25 percent, respectively, of an acid addition salt of distilled cocoa amine, said mixture having an iodine value of less than 12.

7. A froth flotation composition comprising a pulp composed of comminuted sylvanite ore suspended in a brine saturated with the constituents of said ore; and admixed therewith, a cationic sylvite collector composed of a mixture of 70 percent by weight of an acid addition salt of hydrogenated distilled tallow amine and 30 percent of an acid addition salt of distilled cocoa amine, said mixture having an iodine value of less than 12; and said mixture being employed in an amount of 0.07 to 0.16 pound per ton of said ore.

8. A froth flotation composition comprising a pulp composed of a comminuted sylvanite ore suspended in a brine saturated with the constituents of said ore; and admixed therewith, a cationic sylvite collector composed of a mixture of acid addition salts of the primary unbranched saturated and olefinically unsaturated aliphatic amines, caprylyl amine, capryl amine, lauryl amine, myristyl amine, palmityl amine, stearyl amine, oleyl amine, and linoleyl amine in percentages by weight, respectively, of about 1.5 percent, 1.8 percent, 13.5 percent, 6.0 percent, 25.1 percent, 46.6 percent, 5.2 percent and 0.3 percent; said mixture having an iodine value of less than 12; and said mixture being employed in an amount by weight of 0.07 to 0.16 pound per ton of said comminuted sylvanite ore.

9. A process for separating sylvite values from pulp formed of particles of comminuted sylvanite ore suspended in a brine saturated with the constituents of said ore that comprises subjecting said pulp to froth flotation employing a cationic sylvite collector composed of a mixture of 60 percent to 80 percent by weight of an acid addition salt of hydrogenated tallow amine and 40 percent to 20 percent, respectively, of an acid addition salt of distilled cocoa amine, said mixture having an iodine value of less than 12.

45

#### References Cited by the Examiner

##### UNITED STATES PATENTS

|           |         |        |       |           |
|-----------|---------|--------|-------|-----------|
| 2,355,365 | 8/1944  | Cole   | ----- | 209—166   |
| 2,689,649 | 9/1954  | Atwood | ----- | 209—166   |
| 2,695,100 | 11/1954 | Barr   | ----- | 209—166   |
| 2,772,775 | 12/1956 | Atwood | ----- | 209—166 X |

##### OTHER REFERENCES

Noller, C. R., Chem. of Org. Compds., W. B. Saunders Co., OD 253 N 65 Phila. 1955 (p. 179).

HARRY B. THORNTON, Primary Examiner.

R. HALPER, Assistant Examiner.